

## UNITED STATES PATENT OFFICE.

HANS T. CLARKE AND CARL J. MALM, OF ROCHESTER, NEW YORK, ASSIGNORS TO EAST-MAN KODAK COMPANY, OF ROCHESTER, NEW YORK, A CORPORATION OF NEW YORK.

PROCESS OF MAKING CELLULOSIC ESTERS CONTAINING HALOGEN-SUBSTITUTED FATTY-ACID GROUPS.

No Drawing.

Application filed January 18, 1928. Serial No. 247,742.

This invention relates to processes of making cellulosic esters containing halogen-substituted fatty acid groups. One object of the invention is to provide a simplified and relatively inexpensive process for making such esters by a single reaction. Other objects will hereinafter appear.

We have found that such esters may be made by subjecting cellulosic material to the coaction of a halogen-substituted fatty acid containing more than five carbon atoms and an organic acid anhydrid which impels this esterification but does not itself contribute any cellulose esterifying groups to the product. Moreover, the anhydrid is converted into an acid which does not contribute any groups to the ester.

The presence of substituted halogens in fatty acids either retards or prevents the formation of cellulose esters of such acids under conditions which will form useful or substantially undegraded esters. When the fatty acid contains five carbon atoms or less, the inhibiting effect of the halogen, whether the latter be in the alpha or other position, prevents esterification for all practical purposes. But when the halogen-substituted fatty acids contain more than five carbon atoms, useful cellulose esters containing them can be prepared by our process by a single reaction. The length of the carbon chain is thus the determining factor and not the alpha or other position of the halogen atoms. The greater the number of carbon atoms, provided there are more than five, the more readily can the esterification be brought about in spite of the opposing effect of the halogen atoms. For example, halogen-substituted stearic acid is readily esterified with cellulose by our process, while halogen-substituted caproic acid is esterified more slowly. The intermediate members of the halogen-substituted fatty acid series, such as halogen-substituted heptylic, caprylic, pelargonic, capric, lauric, myristic, palmitic and margaric acids can be esterified with cellulose with intermediate ease of reaction. Of the halogen-substituted higher fatty acids which we can employ, we prefer to select the mono, di, tri or tetra brom or chlor members of the series. The corresponding iodine compounds are expensive.

For the anhydrid which impels esterification, without itself adding any groups to the ester, we prefer monochloroacetic anhydrid. 55 This is the least expensive and the most readily prepared of the halogen-substituted fatty acid anhydrids having less than ten carbon atoms. But there can be employed the di and trichloroacetic anhydrids, as well as 60 the mono, di and tribromacetic anhydrids, or mixtures of them. The reaction can be carried out using mono, di and trichlor and brom propionic and butyric anhydrids. But they are relatively too expensive, without any 65 compensating advantage. Likewise the corresponding iodine-substituted acetic, propionic and butyric anhydrids cost too much. But anhydrids other than halogen-substituted ones can also be employed, such as 70 methoxy acetic anhydrid and its higher alkyl homologues beginning with ethoxy acetic anhydrid. It is a characteristic of all of the above named anhydrids that they do not contribute groups to the ester. For example, the 75 cellulose esters produced contain no chloroacetic groups when chloroacetic anhydrid is employed, nor any methoxy acetic groups when methoxy acetic anhydrid is used.

As the cellulosic materials to be esterified, 80 we can use any customarily employed in the manufacture of the hitherto known cellulosic esters. For instance, cotton fiber tissue paper, clean cotton, surgical cotton wool, and even bleached sulfite wood pulp are useful 85 These materials, especially the cotton ones, are sufficiently undegraded when they enter the reaction, so that they yield esters of good flexibility. Of course, our process can be applied to the esterification of chemically 90 affected cellulosic materials, such as so-called hydrocellulose, reverted cellulose from the viscose or cuprammonium processes, lower cellulose nitrates, lower ethyl celluloses, etc.

The temperature at which our process is 95 conducted must obviously be above the melting point of the ingredients of the esterifying bath, but it should not rise to a point where the products are degraded, as indicated by the poor quality of films prepared from the 100 resulting esters. The melting points of the esterifying baths are lower than the melting points of the ingredients taken alone. Moreover, the anhydrids which we use have a

strong solvent action upon the acids which are employed, thus tending to insure good working baths. It is convenient, although not essential, to have an additional solvent present which will not enter into the reaction. We have found monochloracetic acid to be useful for this purpose. And as the reaction proceeds, further amounts of monochloracetic acid are formed and likewise add to the fluidity of the bath. Under these circumstances, temperatures between 50° C. and 80° C. are satisfactory, 60° to 65° C. being preferred. The reaction can be hastened and more thorough results obtained when a catalyst is present. We may use any of the customary esterifying catalysts, but we prefer the milder ones, such as the perchlorates disclosed in United States Patent No. 1,645,915, Carl J. Malm, October 18, 1927, process of making cellulose esters of organic acids. Zinc chloride is likewise usable, as well as the red phosphorus and chlorine of United States Patent No. 1,591,590, William R. Webb and Carl J. Malm, July 6, 1926.

We shall now describe several examples of our invention, but it will be understood that the latter is not limited to the illustrative details thus set forth, except as indicated in the appended claims. A reaction bath is prepared by warming at 60° to 65° C. for 1 to 2 hours the following mixture,—8 parts by weight of cellulose, 40 parts by weight of chloracetic anhydrid, 20 parts by weight of chloracetic acid and .05 parts by weight of magnesium perchlorate trihydrate. For convenience we shall hereinafter refer to this as the standard bath. Into this bath there are thoroughly stirred 15 parts by weight of alpha bromo stearic acid and 4 parts by weight of acetic acid. By maintaining a temperature between 60° and 65° C., a clear dope forms in about 6 hours, indicating the completion of the reaction. The product is isolated by pouring into methyl alcohol and washing the precipitate with this same liquid. The cellulose-aceto-alpha-bromo-stearate thus produced contains 11.3% of bromine and is soluble in acetone, chloroform, benzene, or mixtures of these, and can be deposited from its solutions in the form of transparent flexible films which are substantially non-inflammable,—that is, will not burn with a sustained flame when held in the presence of an igniting flame.

In another example of our invention there are stirred into the standard bath hereinabove described 17 parts by weight of 9-10-dibromo stearic acid and 7 parts by weight of acetic acid (this halogen-substituted stearic acid is readily prepared by brominating oleic acid). After about 6 hours at 60° to 65° C. the reaction is complete, as indicated by the formation of a clear homogeneous dope, which is precipitated in methyl alcohol and the product washed with the same substance.

The product contains 23% of bromine, is soluble in acetone, in chloroform and in benzene, or mixtures of these liquids, and deposits from its solutions transparent, flexible and very non-inflammable films.

To the standard bath hereinabove described there may, in still a further example of our invention, be added 12 parts by weight of dichloro stearic acid (obtained by chlorinating oleic acid) and 5 parts by weight of acetic acid. After 6 hours at 60° to 65° C. the clear dope is poured into methyl alcohol with vigorous stirring and the precipitate washed until purified. It contains 8.5% of chlorine and is soluble in acetone and in chloroform, or mixtures of them; but is insoluble in benzene. It yields flexible, transparent films.

In yet a different example of our invention there are added to the standard bath hereinabove described 14 parts by weight of tetrachloro stearic acid and 5 parts by weight of acetic acid (the first-named acid may be prepared by adding chlorine to the acid formed upon saponification of linseed oil). After 6 hours at 60° to 65° C. the solution becomes clear enough and is poured with agitation into methyl alcohol and the precipitate washed with said alcohol. The cellulose aceto-tetrachloro stearate thus produced contains 14% of chlorine and is soluble in acetone and chloroform or mixtures of them, but not in benzene. It forms flexible, transparent films of very low inflammability.

In another example of our invention parts by weight of alpha bromo caproic acid and 4 parts by weight of acetic acid are stirred into the standard bath hereinabove described. This is heated at 60° to 65° C. until a clear dope is obtained, the product being isolated by precipitating in and washing with methyl alcohol. The purified cellulose aceto-alpha-bromo caproate contains 5% of bromine and is soluble in chloroform.

The above described products and others produced by our process yield flexible films or filaments without softeners or plastifiers, but chloroform-soluble or acetone-soluble plastifiers or softeners heretofore used with cellulose acetates may be employed with them, triphenyl and tricresyl phosphates being examples of the large number that can be employed. Our compounds can be mixed or laminated with cellulose nitrate or acetate by means of a common solvent. Films of them can be backed with a cellulose acetate layer or with hygroscopic nitrocellulose coatings to prevent static, or nitrocellulose or acetate films may be backed with thin layers of our compounds. In short, our process can produce products of technical importance in the preparation of films for photographic purposes, filaments for rayon, lacquers, artificial leather, moldable plastics, etc.

Having thus described our invention, what we claim as new and desire to secure by Letters Patent is:

1. In the process of making cellulosic esters containing halogen-substituted fatty acid groups, subjecting cellulosic material to the coaction of a halogen substituted fatty acid containing more than five carbon atoms and an organic acid anhydrid which impels such esterification but is free from cellulose-esterifying groups and during the esterification is converted into a compound that is also free from cellulose-esterifying groups.
  2. In the process of making cellulosic esters containing halogen-substituted fatty acid groups, treating cellulosic material with an esterifying bath containing a halogen-substituted fatty acid having more than five carbon atoms and a halogen-substituted fatty acid anhydrid having less than ten carbon atoms.
  3. In the process of making cellulose esters
- containing halogen-substituted fatty acid groups, treating cellulosic material with an esterifying bath containing a halogen-substituted fatty acid having more than five carbon atoms, and chloracetic anhydrid. 25
4. In the process of making cellulosic esters containing a halogen-substituted stearic acid group, subjecting cellulosic material to the coaction of a corresponding halogen-substituted stearic acid and a halogen-substituted fatty acid anhydrid having less than ten carbon atoms. 30
5. In the process of making a cellulose ester containing a brom-substituted stearic acid group, treating cellulosic material in a bath containing brom-substituted stearic acid and chloracetic anhydrid. 35

Signed at Rochester, New York, this 10th 40  
day of January, 1928.

HANS T. CLARKE.  
CARL J. MALM.